

## UNITED STATES PATENT OFFICE

2,363,104

## MAGNESITE ORE TREATMENT

Arthur J. Weinig, Golden, Colo., assignor to Basic  
Magnesium, Incorporated, Las Vegas, Nev., a  
corporation of Nevada

No Drawing. Application April 26, 1943,  
Serial No. 484,633

25 Claims. (Cl. 209—166)

This invention relates to the froth flotation treatment of magnesite ores for the recovery of the magnesite content of the ore separate from other ore constituents.

The present application contains subject matter related to the disclosures in the following co-pending applications I have filed:

Serial No. 394,851, filed May 23, 1941, for Separation of magnesite ore constituents; Serial No. 430,619, filed February 12, 1942, for Treatment of magnesite ores; Serial No. 458,323, filed September 14, 1942, for Flotation of magnesite; and Serial No. 474,982, filed February 6, 1943, for Froth flotation treatment of low grade magnesite ores.

Features described but not claimed herein have been made the subjects matter of claims in my aforesaid applications. In addition, the present application claims certain features partially disclosed in the first mentioned application, but which could not be claimed in said application without introducing new matter therein, and as to such features the present application is a substitute for said earlier filed application.

Magnesite ores occur in numerous deposits, such as the one at Luning, Nevada, and consist of magnesium carbonate compositions containing as contaminants one or more of the following: dolomite, serpentine, forsterite, hydromagnesite and similar compositions. For the present consideration, these ores are classified according to their magnesium oxide content, lime content and insoluble (silica and gangue) content.

For certain industrial purposes, a product of suitable market grade will contain not to exceed 1.5% CaO and not to exceed 0.75% insoluble. When relatively high grade ores are treated, various methods may be employed to bring the final product within the desired grade. Of these, froth flotation concentration has proved highly

satisfactory, but when lower grade ores are subjected to froth flotation, the methods heretofore known are not effective in making a product of the prescribed grade.

5 In my earlier investigations, I have discovered that the magnesite content of such magnesite ores can be separated cleanly from lime-bearing constituents such as dolomite, or insolubles such as serpentine, by forming a colloidal metallic hydroxide precipitate in the pulp of the treatment by the reaction of certain types of metallic salts with the lime-bearing minerals in the circuit.

15 This colloidal precipitate which I have chosen to call a "non-acid hydrogel" acts as a depressant for the lime-bearing and other contaminant matter permitting various collector reagents to function efficiently in such a pulp and concentrate the magnesite content in the pulp with only 20 a nominal amount of lime and insoluble constituents present.

25 A variety of metallic salts were tested and found to be satisfactory for this purpose. In general, salts of iron, tin and aluminum were quite satisfactory, and where the alkalinity of the circuit did not afford sufficient material for the above reaction, I added caustic, such as caustic soda or potash, to the circuit to insure a 30 reaction of the desired character. Because of their generally satisfactory qualities and relatively low cost, ferric chloride and aluminum sulfate have been preferred reagents in these treatments, although tin chloride and ferrous sulfate have been used to some extent, as well.

35 The collector reagents of such treatments were fatty acid compositions, such as oleic, palmitic, stearic, capric and lauric acids or the like, and their salts, such as coconut oil soap, palm kernel oil soap, pure sodium oleate, and the like. With

these, certain frothers were employed in some tests and pine oil and synthetic alcohol compositions were found to be well suited for this purpose.

Further investigations led to the discovery that fractionation flotation would afford a recovery of a substantial percentage of the magnesite content. One typical test operation will suffice to illustrate this stage of the development. The ore taken for test was from a Luning, Nevada deposit and analyzed as follows:

|                                     | Per cent analysis |      |       |
|-------------------------------------|-------------------|------|-------|
|                                     | Insoluble         | CaO  | MgO   |
| 1 Chalky white vein matter          |                   | 4.16 | 39.45 |
| 2 White crystalline vein matter     |                   | 0.24 | 47.27 |
| 3 Dark gray crystalline vein matter | 0.72              | 0.56 | 46.87 |
| 4 Ore as taken for test             | 2.04              | 1.76 | 44.60 |

300 grams of said ore was ground to -100 mesh and introduced into 2000 ml. of water. The reagent materials selected were 5 ml. of 10%  $\text{FeCl}_3$  solution, 0.10 gram KOH, and 0.30 ml. of 50% lauric acid. After an initial froth was formed and collected an additional 0.10 ml. lauric acid was added and a second froth collected. Still another 0.10 ml. lauric acid was introduced into the pulp residue and a final froth formed and was collected. The results of these operations were as follows:

|           | Per cent analysis |                 |        |      |
|-----------|-------------------|-----------------|--------|------|
|           | Weight            | Per cent weight | Insol. | CaO  |
| 1st froth | 180               | 60              | 0.64   | 1.24 |
| 2nd froth | 35                | 11.7            | 1.20   | 1.44 |
| 3rd froth | 26                | 8.3             | 2.12   | 2.04 |

It will be noted that the ore taken for the aforesaid test was of relatively high grade and the formation of the hydrogel alone was sufficient to depress enough of the lime and insoluble content to permit recovery of a substantial proportion of the magnesite content of desired grade. However, when lower grade and more mineralogy complex ores are subjected to treatment, other means of inhibiting the flotation of undesirable constituents must be provided to hold the lime and insoluble content of the concentrate within prescribed limits.

Thus, in my application Serial No. 430,619 I disclosed that beneficial results could be obtained by the inclusion in a treatment of the above described character of a molecularly dehydrated phosphate or salt of phosphoric acid. Tetra alkali pyrophosphate compositions and alkali tetraphosphates were cited as classes of compositions suitable for this purpose.

In addition, this application disclosed that the caustic of the treatment might be either a hydroxide, or a basic salt; the latter term being used in the sense of "having the base-forming constituents present in excess of the proportion necessary for a normal compound." It was disclosed additionally that an alkali circuit was not essential as good results were obtained with a

pH of 6 or slightly higher, provided basic salts or hydroxides are formed.

The pyrophosphate compositions were found to be particularly effective in retarding the passage of contaminant slimes into the froth and since such slimes are frequently formed in substantial quantities in milling operations of this character, the lesser amount of the slimes entering the concentrate not only improved grade and recovery but had the added benefit of maintaining the circuit in a condition of efficient equilibrium.

The next phase of the development came about as a result of war shortages. Supplies of coconut oil soap and palm kernel oil soap were cut off necessitating substitution of other collector reagents in the operations hereinbefore described. The class of compositions designated generally as naphthenic acids and salts thereof comprising any one or combination of non-benzenoid cyclic carboxylic acids derived from petroleum were investigated, and found to give highly satisfactory results.

Again when such reagents were used, the non-acid hydrogen was formed by reacting the metallic salt with alkaline material of the circuit and preferably a pyrophosphate composition was used in conjunction therewith to offset the tendency of the naphthenic acid collector to carry lime-bearing constituents and particularly slimes into the froth. This development has been made the subject matter of my copending application Serial No. 458,323.

A typical test operation involving each of the aforesaid treatments will be cited to illustrate the progressive efficiency of the development. In the first of these tests, ore from a Luning, Nevada deposit was crushed to a 5 inch maximum size and passed over a 2½ inch screen. The part of the ore not passing the screen was handpicked and the low grade portion was remixed with the minus 2½ inch portion.

This mixture containing a relatively high proportion of slimy contaminant, was ground to -100 mesh. A suitable pulp was formed of the ground product and subjected to froth flotation with the following reagents:

|                  | Lbs. per ton |
|------------------|--------------|
| Aluminum sulfate | 8.4          |
| Caustic soda     | 2.62         |
| Lauric acid      | 3.14         |

The pH of the pulp after addition of the reagent was determined as 8.3. The pilot mill results of the tests are shown below:

|             | Product | Rate          | Percent | Percent | Percent |
|-------------|---------|---------------|---------|---------|---------|
|             |         |               | of feed | insol.  | CaO     |
| Feed        |         | Lbs. per hour | 189     | 100     | 2.28    |
| Concentrate |         |               | 81      | 43      | 0.62    |
| Tailing     |         |               | 108     | 57      | 3.51    |

In the next test the ore taken for treatment was ore from the Margie claim, Luning, Nevada, assaying 2.21% insoluble and 4.41% CaO, and was ground to 100 mesh. A pulp was formed and conditioned with 8 lbs. ferric chloride, 1.5 lbs. tetrasodium pyrophosphate and 1.6 lbs. of #270 naphthenic acid per ton of ore treated.

This mixture, after the initial conditioning, was subjected to froth flotation and a recovery of 47% was obtained. The concentrate analyzed 0.91% insoluble and 1.23% CaO. It should be noted that although the ore taken for this test was relatively low grade, the concentrate formed

in the operation contained considerably less than the prescribed limits of impurities.

The next phase of the development involved the separation of high grade magnesite from dolomite and low grade magnesite constituents of a magnesite ore. To accomplish this result, a hydrogel is formed in the pulp in the manner hereinbefore described. A pyrophosphate composition is used as a depressant for the lime content, and starch is added to depress the insoluble and gangue content which tends to collect in the froth under the action of the naphthenic acid or lauric acid collector reagent.

The details of the aforesaid operation are described in my copending application, Serial No. 474,982, and represent the culmination of my developments in the treatment of magnesite ores, prior to the present invention.

While the aforesaid methods are effective in the treatment of many grades of magnesite ores, they will not produce the desired grade of concentrate when certain low grade ores are treated. The present invention resides in the discovery that silicic acids may be used in conjunction with such treatments to produce a highly selective froth of low volume with flotation of lime-bearing minerals and gangue slimes effectively retarded.

It is an object of the present invention to provide a simple, economical and efficient method of concentrating the magnesite content of magnesite ores in an action in which only fractional amounts of insoluble and gangue matter collect in the concentrate.

Another object of the present invention is to provide a froth flotation treatment for magnesite ores in which reagent costs are substantially reduced without impairing metallurgical efficiency.

Other objects reside in novel steps and treatments, the details of which will be explained in the course of the following description.

A typical treatment embodying the features of the present invention involves the use of the following preferred reagent combination, designated in pounds reagent per ton of ore:

(a) Salts of aluminum and iron, such as aluminum sulfate and ferric chloride—3 to 16 lbs./ton;

(b) Naphthenic acids or lauric acids—0.3 to 4 lbs./ton;

(c) Tetra alkali pyrophosphate—0.1 to 3 lbs./ton;

(d) Causticized starch—0.3 to 2 lbs./ton;

(e) Silicic acids—0.5 to 3 lbs./ton.

In performing the process, the ore is ground and mixed with water to form a free-flowing pulp, and this pulp is subjected to a froth flotation treatment in the presence of the reagents. In an operation of this type, each of the above enumerated reagent materials functions in the manner hereinafter to be described.

The salts of aluminum or iron are added to the pulp preferably ahead of the flotation circuit, and are conditioned by agitation until reaction is complete. In this operation the salts are decomposed by the lime-bearing mineral grains of the ore, resulting in a surface deposition on such grains of hydrates of the metals in the salts. In this reaction, aluminum and iron are precipitated out of solution and equivalent amounts of lime are rendered soluble.

The effect of the reaction is to prevent the flotation of lime-bearing minerals by the inhibiting effect of the deposited hydrate. More specifically, such salts have been found to possess special affinity for dolomite, calcite and similar

calcareous materials, but have no affinity for magnesite. The reaction apparently proceeds according to the following equation:



The naphthenic acids and lauric acids recommended for this treatment function in the pulp as both frothing and collecting agents. They exert a strong flotation effect on the magnesite ore constituents and will float calcite and dolomite readily as well as gangue materials unless said constituents are subjected to satisfactory inhibiting influences. Consequently, when the hydrate deposit is formed on the lime-bearing mineral surfaces, the reagents function to produce a desirable concentration, particularly when the ores are of relatively high grade.

As the ores become poorer in grade, it will be necessary to further depress or exert a flotation inhibiting effect on the gangue and lime-bearing minerals. To assist in this action, the tetra alkali pyrophosphate compositions are introduced in the pulp conditioning stage and further inhibit the flotation of lime-bearing constituents. However, these compositions have some tendency to cause flotation of gangue matter and insoluble silicates.

Consequently, when an ore of relatively low grade contains substantial quantities of insoluble silicates, it is necessary to add to the reagents hereinbefore designated, some additional agent which will inhibit the flotation of the siliceous material. Causticized starch was found to be an effective addition agent for this purpose. It overcomes the flotation tendency of mineral silicates due to the presence of tetra alkali pyrophosphate and also reduces the toughness and volume of froth. For many flotation treatments the combination of the aforesaid reagents is ample to attain the desired results.

However, when still lower grade ores are to be treated and the aforesaid reagent combination will not produce satisfactory results, a concentrate of prescribed grade can be attained by including silicic acids as an additional reagent in the treatment. More specifically, the silicic acid composition should be a polymerized acid which is not an ionized salt, or acid or gel. Preferably, such composition is produced by exactly neutralizing alkali silicates with mineral acid and then aging.

The inclusion of the silicic acids in the treatment thus provides a low cost reagent which is effective in producing a highly selective froth of low volume. It aids in retarding the flotation of lime-bearing minerals and gangue slimes and gives improved recovery and grade in the magnesite concentrates. Further, in many treatments it will supplant the use of the tetra alkali pyrophosphate.

A typical test operation will illustrate the advantage gained by introducing a quantity of silicic acid into the treatment. A sample of Gabbs Valley ore ground dry to pass through 100 mesh and containing 20% plus 200 mesh by weight was used in the test. The analysis of the ore was as follows:

|                                                | Per cent |
|------------------------------------------------|----------|
| Insoluble                                      | 3.18     |
| Lime (CaO)                                     | 5.98     |
| $\text{R}_2\text{O}_3$ group                   | 1.09     |
| Iron (Fe)                                      | 0.59     |
| 500 grams of the ore mixed with 2.5 grams alu- |          |

minum sulfate was agitated in a laboratory mechanical type flotation machine with 2 liters of water heated to 130° F. This yielded a pulp at a temperature of 100° F. Other reagents were added to the pulp in the following order: (1) causticized starch, (2) silicic acid, (3) tetrasodium pyrophosphate, and (4) naphthenic acids.

After one minute conditioning, air was admitted to the cell and froth drawn off for two minutes. The slimes from the concentrate were 10

TEST B (STANDARD REAGENT COMBINATION)  
Reagents used (equivalent lb. per ton of head ore)

|                                | Roughing | Cleaning |
|--------------------------------|----------|----------|
| 5                              |          |          |
| Aluminum sulfate.....          | 10.0     | None     |
| Causticized starch.....        | 0.4      | 0.4      |
| Silicic acid.....              | 1.4      | 0.4      |
| Tetrasodium pyrophosphate..... | 0.6      | 0.4      |
| Naphthenic acids.....          | 0.58     | None     |

| Product                | Weight |          |               | Analysis |       |                               |               |      |                               |
|------------------------|--------|----------|---------------|----------|-------|-------------------------------|---------------|------|-------------------------------|
|                        | G.     | Per cent | Cum. per cent | Per cent |       |                               | Cum. per cent |      |                               |
|                        |        |          |               | Insol.   | CaO   | R <sub>2</sub> O <sub>3</sub> | Insol.        | CaO  | R <sub>2</sub> O <sub>3</sub> |
| 1st cleaner froth..... | 263    | 52.6     | 52.6          | .58      | 1.41  | .46                           | .58           | 1.41 | .46                           |
| 2nd cleaner froth..... | 27     | 5.4      | 58.0          | .97      | 3.25  | .54                           | .60           | 1.57 | .47                           |
| Cleaner tailing.....   | 89     | 17.8     | 75.8          | 3.54     | 10.37 | 1.08                          | 1.29          | 3.64 | .61                           |
| Rougher tailing.....   | 121    | 24.2     | 100.0         | 9.38     | 12.92 | 2.98                          | 3.25          | 5.89 | 1.18                          |

returned to the machine and after mixing, a second froth was drawn off for one and one-half minutes. This procedure was repeated two more times and the slime from the last frothing operation was not returned to the machine.

The rougher concentrate was returned to the machine with the water decanted from the rougher tailing and after the addition of necessary reagents was subjected to cleaning for from five to six minutes. Whenever it was desired to raise the froth level, the nearly clear water was decanted off the concentrates and returned to the machine.

The silicic acid of the treatment was prepared by the addition of 1.8 ml. 50% sulfuric acid to 10 ml. water glass (41° Bé. Ratio Na<sub>2</sub>O to SO<sub>2</sub> 1 to 3.25) diluted to 200 ml. with water and aged for four to five days before use.

In order to illustrate the effect of silicic acid in the aforesaid treatments, the same ore was 25 treated under similar conditions using the same combination of reagents except that silicic acid was omitted. The results of this testing are set forth in the following tabulation:

## TEST C (SILICIC ACID OMITTED)

Reagents used (equivalent lb. per ton of head ore)

|                                | Roughing | Cleaning |
|--------------------------------|----------|----------|
| 35                             |          |          |
| Aluminum sulfate.....          | 10.0     | None     |
| Causticized starch.....        | 0.4      | 0.4      |
| Silicic acid.....              | None     | None     |
| Tetrasodium pyrophosphate..... | 0.6      | 0.6      |
| Naphthenic acids.....          | 0.73     | None     |

40

| Product                | Weight |          |               | Analysis |       |                               |               |      |                               |
|------------------------|--------|----------|---------------|----------|-------|-------------------------------|---------------|------|-------------------------------|
|                        | G.     | Per cent | Cum. per cent | Per cent |       |                               | Cum. per cent |      |                               |
|                        |        |          |               | Insol.   | CaO   | R <sub>2</sub> O <sub>3</sub> | Insol.        | CaO  | R <sub>2</sub> O <sub>3</sub> |
| 1st cleaner froth..... | 179    | 35.6     | 35.6          | 0.82     | 3.04  | .52                           | .82           | 3.04 | .52                           |
| 2nd cleaner froth..... | 93     | 18.5     | 54.1          | 0.80     | 2.11  | .50                           | .81           | 2.72 | .52                           |
| Cleaner tailing.....   | 109    | 21.7     | 75.8          | 2.26     | 6.12  | .86                           | 1.23          | 3.70 | .62                           |
| Rougher tailing.....   | 122    | 24.2     | 24.2          | 8.98     | 12.70 | 2.88                          | 3.10          | 6.87 | 1.17                          |

The test results follow:

## TEST A (STANDARD REAGENT COMBINATION)

Reagents used (equivalent lb. per ton of head ore)

|                                | Roughing | Cleaning |
|--------------------------------|----------|----------|
| Aluminum sulfate.....          | 10.0     |          |
| Causticized starch.....        | 0.4      | 0.4      |
| Silicic acid.....              | 1.4      | 0.4      |
| Tetrasodium pyrophosphate..... | 0.6      | 0.4      |
| Naphthenic acids.....          | 0.73     |          |

The peculiarity of this test is that the second 65 froth is of better grade than the first one. This is probably due to the fact that the first froth contained more low grade slime.

60

| Product                | Weight |          |               | Analysis |       |                               |               |      |                               |
|------------------------|--------|----------|---------------|----------|-------|-------------------------------|---------------|------|-------------------------------|
|                        | G.     | Per cent | Cum. per cent | Per cent |       |                               | Cum. per cent |      |                               |
|                        |        |          |               | Insol.   | CaO   | R <sub>2</sub> O <sub>3</sub> | Insol.        | CaO  | R <sub>2</sub> O <sub>3</sub> |
| 1st cleaner froth..... | 275    | 55.4     | 55.4          | .47      | 1.49  | .44                           | .47           | 1.49 | .44                           |
| 2nd cleaner froth..... | 35     | 7.0      | 62.4          | .79      | 2.31  | .56                           | .51           | 1.59 | .45                           |
| Cleaner tailing.....   | 101    | 20.3     | 82.4          | 3.74     | 14.77 | 1.18                          | 1.31          | 4.84 | .63                           |
| Rougher tailing.....   | 86     | 17.3     | 100.0         | 12.52    | 10.67 | 4.12                          | 3.24          | 5.84 | 1.24                          |

## TEST D (TETRASODIUM PYROPHOSPHATE OMITTED)

Reagents used (equivalent lb. per ton of head ore)

|                                | Roughing | Cleaning |
|--------------------------------|----------|----------|
| Aluminum sulfate.....          | 10.0     | None     |
| Causticized starch.....        | 0.4      | 0.4      |
| Silicic acid.....              | 1.4      | 0.4      |
| Tetrasodium pyrophosphate..... | None     | None     |
| Naphthenic acids.....          | 0.58     | None     |

(3) 2d cleaning (with pyro and other gangue depressant) eliminated 78% insoluble and 71% of the lime content of the first cleaner concentrate.

5 The ratio of insoluble elimination to lime elimination in successive operations is then as follows:

|                                                |     |
|------------------------------------------------|-----|
| Roughing (no pyro).....                        | 2.4 |
| 1st cleaning (pyro alone).....                 | 0.8 |
| 2d cleaning (pyro with other depressants)..... | 1.1 |

These figures confirm the general impression

| Product                | Weight |          |               | Analysis |       |                               |               |      |                               |
|------------------------|--------|----------|---------------|----------|-------|-------------------------------|---------------|------|-------------------------------|
|                        | G.     | Per cent | Cum. per cent | Per cent |       |                               | Cum. per cent |      |                               |
|                        |        |          |               | Insol.   | CaO   | R <sub>2</sub> O <sub>3</sub> | Insol.        | CaO  | R <sub>2</sub> O <sub>3</sub> |
| 1st cleaner froth..... | 267    | 53.4     | 53.4          | .47      | 1.49  | .42                           | .47           | 1.49 | .42                           |
| 2nd cleaner froth..... | 26     | 5.2      | 58.6          | .82      | 3.49  | .42                           | .49           | 1.67 | .42                           |
| Cleaner tailing.....   | 94     | 18.8     | 77.4          | 3.82     | 12.92 | 1.06                          | 1.31          | 4.40 | .57                           |
| Rougher tailing.....   | 113    | 22.6     | 100.0         | 9.72     | 10.67 | 3.21                          | 3.21          | 5.82 | 1.17                          |

In order to summarize the results of the preceding tests A, B, C and D, the grade of a concentrate containing 55% of the heads by weight has been calculated by interpolation.

|                                                           | Analysis of concentrate by interpolation for 55% weight recovery |      |                               |  |
|-----------------------------------------------------------|------------------------------------------------------------------|------|-------------------------------|--|
|                                                           | Insol.                                                           | CaO  | R <sub>2</sub> O <sub>3</sub> |  |
|                                                           |                                                                  |      |                               |  |
| Standard reagent combination (mean of tests A and B)..... | 0.53                                                             | 1.48 | 0.45                          |  |
| Silicic acid omitted (test C).....                        | 0.81                                                             | 2.72 | 0.52                          |  |
| Tetrasodium pyrophosphate omitted (test D).....           | 0.47                                                             | 1.55 | 0.42                          |  |

In order to bring out the effect of the tetrasodium pyrophosphate on the various classes of gangues, the following test (E) is reported in which two cleaning stages were employed.

## TEST E

Reagents used (equivalent lb. per ton of head ore)

|                                | Roughing | 1st cleaning | 2nd cleaning |
|--------------------------------|----------|--------------|--------------|
| Aluminum sulfate.....          | 10.0     | None         | None         |
| Causticized starch.....        | 0.4      | None         | 0.32         |
| Silicic acid.....              | 1.4      | None         | 0.4          |
| Tetrasodium pyrophosphate..... | None     | 0.8          | 0.4          |
| Naphthenic acids.....          | 0.58     | 0.22         | 0.36         |

| Product                  | Weight |          |               | Analysis |       |                               |               |      |                               |
|--------------------------|--------|----------|---------------|----------|-------|-------------------------------|---------------|------|-------------------------------|
|                          | G.     | Per cent | Cum. per cent | Per cent |       |                               | Cum. per cent |      |                               |
|                          |        |          |               | Insol.   | CaO   | R <sub>2</sub> O <sub>3</sub> | Insol.        | CaO  | R <sub>2</sub> O <sub>3</sub> |
| Cleaner froth.....       | 212    | 42.4     | 42.4          | 0.31     | 1.16  | 0.40                          | 0.31          | 1.16 | 0.40                          |
| 2d cleaner tailing.....  | 120    | 24.0     | 66.4          | 1.88     | 5.07  | 0.84                          | 0.87          | 2.68 | 0.56                          |
| 1st cleaner tailing..... | 91     | 18.2     | 84.6          | 2.84     | 13.80 | 1.20                          | 1.30          | 5.00 | 0.70                          |
| Rougher tailing.....     | 77     | 15.4     | 100.0         | 13.64    | 10.43 | 4.82                          | 3.19          | 5.84 | 1.33                          |

The relative amounts of insoluble and lime eliminated by each successive flotation step have been calculated to be as follows:

(1) Roughing (without pyro) eliminated 66% insoluble and 28% lime from the head ore.

(2) 1st cleaning (with pyro alone) eliminated 47% insoluble and 59% lime from the rougher concentrate.

70 The rougher concentrate was returned to the machine with the water decanted from the rougher tailing and, after the addition of necessary reagents, subjected to cleaning for five to six minutes. Whenever it was desired to raise the froth level, the water decanted off the concentrates was returned to the machine.

The results of these tests follow:

| Test No. | Reagents<br>(equiv. lb. per ton of ores) |        |              |              |             | Product | Weight analysis (per cent) |          |        |      |                               |      |
|----------|------------------------------------------|--------|--------------|--------------|-------------|---------|----------------------------|----------|--------|------|-------------------------------|------|
|          | FeCl <sub>3</sub>                        | Starch | Silicic acid | Sodium pyro. | Lauric acid |         | G.                         | Per cent | Insol. | CaO  | R <sub>2</sub> O <sub>3</sub> |      |
| M        | STANDARD REAGENT COMBINATION             |        |              |              |             |         | Concentrate                | 228      | 45.9   | 0.62 | 1.10                          | 0.36 |
|          | 10                                       | 0.4    | 0.2          | 0.6          | 0.92        |         | Cl. tailing                | 112      | 22.5   | 2.54 | 7.70                          | 0.85 |
|          |                                          | 0.4    | 1.4          |              |             |         | R. tailing                 | 157      | 31.6   | 7.30 | 10.45                         | 2.54 |
|          |                                          |        |              |              |             |         | Heads                      | 497      |        | 3.17 | 5.54                          | 1.16 |
| N        | STANDARD REAGENT COMBINATION             |        |              |              |             |         | 1st froth                  | 284      | 57.1   | 0.62 | 1.70                          | 0.43 |
|          | 10                                       | 0.4    | 0.1          | 0.6          | 1.15        |         | 2d froth                   | 23       | 4.6    | 0.88 | 2.55                          | 0.46 |
|          |                                          | 0.4    | 1.4          |              |             |         | Cl. tailing                | 75       | 15.1   | 3.75 | 13.00                         | 1.12 |
|          |                                          |        |              |              |             |         | R. tailing                 | 115      | 23.2   | 8.86 | 11.85                         | 3.18 |
| O        | SODIUM PYROPHOSPHATE OMITTED             |        |              |              |             |         | Heads                      | 497      |        | 3.03 | 5.80                          | 1.18 |
|          | 10                                       | 0.4    | 0.4          | None         | 0.46        |         | Concentrate                | 248      | 49.6   | 0.68 | 1.77                          | 0.28 |
|          |                                          | 0.4    | 1.4          | None         |             |         | Cl. tailing                | 126      | 25.2   | 2.44 | 8.85                          | 0.86 |
|          |                                          |        |              |              |             |         | R. tailing                 | 126      | 25.2   | 8.88 | 10.90                         | 3.06 |
| P        | CAUSTICIZED STARCH OMITTED               |        |              |              |             |         | Heads                      | 500      |        | 3.20 | 5.84                          | 1.13 |
|          | 10                                       | None   | 0.2          | 0.6          | 0.23        |         | 1st froth                  | 229      | 46.1   | 0.71 | 2.15                          | 0.36 |
|          |                                          | None   | 1.4          |              | 0.57        |         | 2d froth                   | 96       | 19.3   | 1.13 | 3.45                          | 0.45 |
|          |                                          |        |              |              |             |         | Cl. tailing                | 58       | 11.7   | 4.10 | 11.80                         | 1.33 |
| Q        | CAUSTICIZED STARCH OMITTED               |        |              |              |             |         | R. tailing                 | 114      | 22.9   | 9.22 | 10.80                         | 3.12 |
|          | 10                                       | None   | 0.2          | 0.6          | 0.86        |         | Heads                      | 497      |        | 3.14 | 5.51                          | 1.13 |
|          |                                          | None   | 1.4          |              |             |         |                            |          |        |      |                               |      |
|          |                                          |        |              |              |             |         |                            |          |        |      |                               |      |
| R        | SILICIC ACID OMITTED                     |        |              |              |             |         |                            |          |        |      |                               |      |
|          | 10                                       | 0.4    | None         | 0.6          | 0.60        |         | 1st froth                  | 227      | 45.5   | 0.70 | 1.67                          | 0.44 |
|          |                                          | 0.4    | None         |              |             |         | 2d froth                   | 42       | 8.4    | 1.26 | 2.88                          | 0.54 |
|          |                                          |        |              |              |             |         | Cl. tailing                | 85       | 17.0   | 2.72 | 9.88                          | 0.86 |
|          |                                          |        |              |              |             |         | R. tailing                 | 145      | 29.1   | 7.54 | 11.60                         | 2.68 |
|          |                                          |        |              |              |             |         | Heads                      | 499      |        | 3.09 | 6.05                          | 1.18 |

As compared with operations in which naphthenic acid was the collector reagent, the use of lauric acid results in a somewhat lower efficiency of separation, permitting the recovery of only 52-54% of the ore by weight instead of 60% obtainable with naphthenic acid. The function of the two reagents was shown to be essentially similar, and omission of each of the three modifying agents (causticized starch, silicic acid and sodium pyrophosphate) resulted in a substantial lowering of the efficiency of the separation.

Lauric acid produces a tougher but less voluminous froth than is produced by naphthenic acid, and the effect of silicic acid as a froth controlling reagent is less apparent. However, the omission of silicic acid from the reagent combination results in a lowering of recovery by some 10% for a given grade of concentrates.

The use of iron salts furnishes additional evidence of the precipitating action on lime-bearing minerals by coloring these minerals in the flotation tailings with a clearly visible rusty stain. The magnesite in the concentrate is unstained.

From the foregoing description of test procedure, it will be apparent that good recoveries will be attained, even when relatively low grade ores

are treated, by following the practice of the present invention. Where practical substitute ingredients have been provided in the reagent combination so that benefit can be taken of price fluctuations or operations continued in the face of critical scarcities without changing the fundamental character of the operation.

In the treatment of low grade ores, the inclusion of silicic acid as an ingredient of the reagent combination becomes important. I am aware that in other operations sodium silicate has been used in the treatment of magnesite ores to form a silica gel in the pulp which precipitates on quartz, serpentine and calcite constituents to depress them. In the present treatment such condition is undesirable and productive of detrimental results, for which reason I have specified herein the essential character of the silicic acid taken for treatment.

A series of tests were undertaken to determine just what characteristics and properties of the silicic acid would give the desired results. In the testing, numerous inconsistencies were noted and after eliminating several possible causes, it was determined that the elapsed time between the preparation of the silicic acid reagent and

its use was critical, with the metallurgical results improving within limits as the age of the prepared reagent increased.

The effect of excess acidity in the reagent also was investigated. These tests demonstrated that a small excess of sulfuric acid used in the preparation of the silicic acid reagent gave the best metallurgical results. Other tests demonstrated that aging the dilute sodium silicate solution before acidification apparently has the same effectiveness as aging the prepared sodium silicate, except that the former method can be completed in much shorter time.

For this reason, I have described the silicic acid as a polymerized acid which is not an ionized salt, acid, or gel, but rather a neutralized and aged silicate composition. While I do not want to be limited to exact proportions in the use of the silicic acid in the reagent combinations of the present invention, I have found that best results are obtained in the treatment when the silicic acid is used in an amount between 0.5 and 3 pounds per ton of ore treated.

The action of the silicic acid composition in the treatment is particularly effective in depressing dolomite, although its functions effectively with other materials such as serpentine, forsterite, hydromagnesite and the like.

The large number of test operations described herein affords a standard of selection of reagent combinations to suit the properties of a given ore taken for treatment. Where reagent ingredients have been described without citation of specific operating data, it will be understood that they are used and function in the treatment in substantially the same way as other ingredients for which they are substitutes.

Changes and modifications may be availed of within the spirit and scope of the invention as defined in the hereunto appended claims.

What I claim and desire to secure by Letters Patent is:

1. The method of concentrating magnetic ores which comprises introducing magnesite ore in finely divided condition into a liquid carrier vehicle to form a pulp, introducing a salt selected from the group consisting of salts of aluminum, tin and iron into said pulp to react with lime-bearing mineral of the pulp and deposit a hydrate of the metal on the surfaces of said lime-bearing mineral, subjecting such pulp to a froth flotation treatment in the presence of a collector reagent selected from the group consisting of oleic, palmitic, stearic, capric, lauric and naphthenic acids and their salts to concentrate the magnesite content of the ore in a froth at the surface of the pulp body, and inhibiting flotation of lime-bearing minerals, siliceous matter and gangue in said pulp under the influence of the collector reagent by having causticized starch and silicic acid present in said pulp.

2. The method of concentrating magnesite ores, which comprises introducing magnesite ore in finely divided condition into a liquid carrier vehicle to form a pulp, introducing a salt selected from the group consisting of salts of aluminum, tin and iron into said pulp to react with lime-bearing mineral of the pulp and deposit a hydrate of the metal on the surfaces of said lime-bearing mineral, subjecting such pulp to a froth flotation treatment in the presence of a collector reagent selected from the group consisting of oleic, palmitic, stearic, capric, lauric and naphthenic acids and their salts to concentrate the magnesite content of the ore in a froth at the surface of the

pulp body, and inhibiting flotation of lime-bearing minerals, siliceous matter and gangue in said pulp under the influence of the collector reagent by having causticized starch and polymerized silicic acid present in said pulp.

3. The method of concentrating magnesite ores, which comprises introducing magnesite ore in finely divided condition into a liquid carrier vehicle to form a pulp, introducing a salt selected from the group consisting of salts of aluminum, tin and iron into said pulp to react with lime-bearing mineral of the pulp and deposit a hydrate of the metal on the surfaces of said lime-bearing mineral, subjecting such pulp to a froth flotation treatment in the presence of a collector reagent selected from the group consisting of oleic, palmitic, stearic, capric, lauric and naphthenic acids and their salts to concentrate the magnesite content of the ore in a froth at the surface of the pulp body, and inhibiting flotation of lime-bearing minerals, siliceous matter and gangue in said pulp under the influence of the collector reagent by having causticized starch, tetra alkali pyrophosphate, and silicic acid present in said pulp.

4. The method of concentrating magnesite ores, which comprises introducing magnesite ore in finely divided condition into a liquid carrier vehicle to form a pulp, introducing a salt selected from the group consisting of salts of aluminum, tin and iron into said pulp to react with lime-bearing mineral of the pulp and deposit a hydrate of the metal on the surfaces of said lime-bearing mineral, subjecting such pulp to a froth flotation treatment in the presence of a collector reagent selected from the group consisting of oleic, palmitic, stearic, capric, lauric and naphthenic acids and their salts to concentrate the magnesite content of the ore in a froth at the surface of the pulp body, and inhibiting flotation of lime-bearing minerals, siliceous matter and gangue in said pulp under the influence of the collector reagent by having causticized starch, tetra alkali pyrophosphate and polymerized silicic acid present in said pulp.

5. The method of concentrating magnesite ores, which comprises introducing magnesite ore in finely divided condition into a liquid carrier vehicle to form a pulp, introducing a salt selected from the group consisting of salts of aluminum, tin and iron into said pulp to react with lime-bearing mineral of the pulp and deposit a hydrate of the metal on the surfaces of said lime-bearing mineral, and subjecting such pulp to a froth flotation treatment during which causticized starch, silicic acid, tetra alkali pyrophosphate and a naphthenic acid collector are successively entered into the pulp.

6. The method of concentrating magnesite ores, which comprises introducing magnesite ore in finely divided condition into a liquid carrier vehicle to form a pulp, introducing a salt selected from the group consisting of salts of aluminum, tin and iron into said pulp to react with lime-bearing mineral of the pulp and deposit a hydrate of the metal on the surfaces of said lime-bearing mineral, and subjecting such pulp into a froth flotation treatment during which causticized starch, silicic acid, tetra alkali pyrophosphate and a lauric acid collector are successively entered into the pulp.

7. The method of concentrating magnesite ores, which comprises introducing magnesite ore in finely divided condition into a liquid carrier vehicle to form a pulp, introducing a salt selected from the group consisting of salts of aluminum,

tin and iron into said pulp to react with lime-bearing minerals of the pulp and deposit a hydrate of the metal on the surfaces of said lime-bearing minerals, and subjecting such pulp to a froth flotation treatment during which caustic starch, silicic acid, and a naphthenic acid collector are successively entered into the pulp.

8. The method of concentrating magnesite ores, which comprises introducing magnesite ore in finely divided condition into a liquid carrier vehicle to form a pulp, introducing a salt selected from the group consisting of salts of aluminum, tin and iron into said pulp to react with lime-bearing minerals of the pulp and deposit a hydrate of the metal on the surfaces of said lime-bearing minerals, and subjecting such pulp to a froth flotation treatment during which caustic starch, silicic acid, and a lauric acid collector are successively entered into the pulp.

9. In the art of concentrating magnesite ores, in which the magnesite content of an aqueous magnesite ore pulp is collected on the surface of the pulp by the action of a collector reagent selected from the group consisting of oleic, palmitic, stearic, capric, lauric and naphthenic acids and their salts in a froth flotation treatment, the improvement which comprises conditioning such magnesite content for selective collection by the reagent in an alkaline medium having a pH of at least 8 by reacting the lime-bearing content of the pulp with a salt selected from the group consisting of salts of aluminum, tin and iron to deposit a hydrate of the metal on the surfaces of the lime-bearing constituents which hydrate prevents such constituents from responding to the action of said collector reagent.

10. In the art of concentrating magnesite ores, in which the magnesite content of an aqueous magnesite ore pulp is collected on the surface of the pulp by the action of a collector reagent selected from the group consisting of oleic, palmitic, stearic, capric, lauric and naphthenic acids and their salts, in a froth flotation treatment, the improvement which comprises conditioning such magnesite content for selective collection by the reagent in an alkaline medium having a pH of at least 8 by reacting the lime-bearing content of the pulp with aluminum sulfate to deposit a hydrate of the metal on the surfaces of the lime-bearing constituents which hydrate prevents such constituents from responding to the action of said collector reagent.

11. In the art of concentrating magnesite ores, in which the magnesite content of an aqueous magnesite ore pulp is collected on the surface of the pulp by the action of a collector reagent selected from the group consisting of oleic, palmitic, stearic, capric, lauric and naphthenic acids and their salts, in a froth flotation treatment, the improvement which comprises conditioning such magnesite content for selective collection by the reagent in an alkaline medium having a pH of at least 8 by reacting the lime bearing content of the pulp with ferric chloride to deposit a hydrate of the metal on the surfaces of the lime-bearing constituents which hydrate prevents such constituents from responding to the action of said collector reagent.

12. In the art of concentrating magnesite ores, in which the magnesite content of an aqueous magnesite ore pulp is colected on the surface of the pulp by the action of a collector reagent selected from the group consisting of oleic, palmitic, stearic, capric, lauric and naphthenic acids and their salts, in a froth flotation treatment, the

improvement which comprises conditioning such magnesite content for selective collection by the reagent in an alkaline medium having a pH of at least 8 by reacting the lime-bearing content of the pulp with a salt selected from the group consisting of salts of aluminum, tin and iron to deposit a hydrate of the metal on the surfaces of the lime-bearing constituents which hydrate prevents such constituents from responding to the action of said collector reagent, and continuing said conditioning treatment until the reaction of the metallic salt is complete, before subjecting said pulp to froth flotation.

13. The method of concentrating magnesite ores, which comprises introducing magnesite ore in finely divided condition into a liquid carrier vehicle to form a pulp, introducing aluminum sulfate into said pulp to react with lime-bearing mineral of the pulp and deposit a hydrate of the metal on the surfaces of said lime-bearing mineral, subjecting such pulp to a froth flotation treatment in the presence of a collector reagent selected from the group consisting of oleic, palmitic, stearic, capric, lauric and naphthenic acids and their salts to concentrate the magnesite content of the ore in a froth at the surface of the pulp body, and inhibiting flotation of lime-bearing minerals, siliceous matter and gangue in said pulp under the influence of the collector reagent by having causticized starch and silicic acid present in said pulp.

14. The method of concentrating magnesite ores, which comprises introducing magnesite ore in finely divided condition into a liquid carrier vehicle to form a pulp, introducing ferric chloride into said pulp to react with lime-bearing mineral of the pulp and deposit a hydrate of the metal on the surfaces of said lime-bearing mineral, subjecting such pulp to a froth flotation treatment in the presence of a collector reagent selected from the group consisting of oleic, palmitic, stearic, capric, lauric and naphthenic acids and their salts to concentrate the magnesite content of the ore in a froth at the surface of the pulp body, and inhibiting flotation of lime-bearing minerals, siliceous matter and gangue in said pulp under the influence of the collector reagent by having causticized starch and silicic acid present in said pulp.

15. The method of concentrating magnesite ores, which comprises introducing magnesite ore in finely divided condition into a liquid carrier vehicle to form a pulp, introducing a salt selected from the group consisting of salts of aluminum, tin and iron into said pulp to react with lime-bearing mineral of the pulp and deposit a hydrate of the metal on the surfaces of said lime-bearing mineral, subjecting such pulp to a froth flotation treatment in the presence of a lauric acid collector reagent to concentrate the magnesite content of the ore in a froth at the surface of the pulp body, and inhibiting flotation of lime-bearing minerals, siliceous matter and gangue in said pulp under the influence of the collector reagent by having causticized starch and silicic acid present in said pulp.

16. The method of concentrating magnesite ores, which comprises introducing magnesite ore in finely divided condition into a liquid carrier vehicle to form a pulp, introducing a salt selected from the group consisting of salts of aluminum, tin and iron into said pulp to react with lime-bearing mineral of the pulp and deposit a hydrate of the metal on the surfaces of said lime-bearing mineral, subjecting such pulp to a froth

flotation treatment in the presence of a naphthenic acid collector reagent to concentrate the magnesite content of the ore in a froth at the surface of the pulp body, and inhibiting flotation of lime-bearing minerals, siliceous matter and gangue in said pulp under the influence of the collector reagent by having causticized starch and silicic acid present in said pulp.

17. In a process for treating magnesite ores for the recovery of magnesite separated from contaminating inclusions, in which magnesite particles of an aqueous magnesite ore pulp are selectively filmed with a collector reagent selected from the group consisting of oleic, palmitic, stearic, capric, lauric and naphthenic acids and their salts, and then the pulp is subjected to froth flotation, the improvement which comprises conditioning the pulp for froth flotation by adding sufficient caustic to the pulp to produce at least a pH of 8, and forming a colloidal metallic hydroxide precipitate in the pulp through the introduction of a metallic salt selected from the group consisting of salts of aluminum, tin and iron into the pulp of the type that will react with the lime content thereof.

18. In a process for treating magnesite ores for the recovery of magnesite separate from contaminating inclusions, in which magnesite particles of an aqueous magnesite ore pulp are selectively filmed with a collector reagent selected from the group consisting of oleic, palmitic, stearic, capric, lauric and naphthenic acids and their salts, and then the pulp is subjected to froth flotation, the improvement which comprises conditioning the pulp for froth flotation by adding sufficient caustic to the pulp to produce at least a pH of 8, and forming a colloidal metallic hydroxide precipitate in the pulp through the introduction of ferric chloride into the pulp.

19. In a process for treating magnesite ores for the recovery of magnesite separate from contaminating inclusions, in which magnesite particles of an aqueous magnesite ore pulp are selectively filmed with a collector reagent selected from the group consisting of oleic, palmitic, stearic, capric, lauric and naphthenic acids and their salts, and then the pulp is subjected to froth flotation the improvement which comprises conditioning the pulp for froth flotation by adding sufficient caustic to the pulp to produce at least a pH of 8, and forming a colloidal metallic hydroxide precipitate in the pulp through the introduction of aluminum sulfate into the pulp.

20. In a process for treating magnesite ores for the recovery of magnesite separate from contaminating inclusions, in which magnesite particles of an aqueous magnesite ore pulp are selectively filmed with a collector reagent selected from the group consisting of oleic, palmitic, stearic, capric, lauric and naphthenic acids and their salts, and then the pulp is subjected to froth flotation, the improvement which comprises conditioning the pulp for froth flotation by forming therein a colloidal metallic hydroxide precipitate through the introduction into the pulp of a metallic salt selected from the group consisting of aluminum, tin and iron of the type that will react with the lime content thereof, and a caustic of the type that will give the pulp a pH of at least 8.

21. The process of treating magnesite ores by froth flotation, which comprises forming a magnesite ore pulp containing high grade magnesite intermixed with a quantity of lime and insoluble constituent particles, and floating high grade

magnesite selectively away from such lime and insoluble contents of the pulp by aerating said pulp in the presence of: a hydrogel-forming salt selected from the group consisting of aluminum, tin and iron salts; silicic acid; causticized starch; a lime depressant selected from the group consisting of alkali pyrophosphates and sodium lignin sulfonate; and a collector reagent selected from the group consisting of oleic, palmitic, stearic, capric, lauric and naphthenic acids and their salts.

22. The process of treating magnesite ores by froth flotation, which comprises forming a magnesite ore pulp containing high grade magnesite intermixed with a quantity of lime and insoluble constituent particles, and floating high grade magnesite selectively away from such lime and insoluble content of the pulp by aerating said pulp in the presence of: a hydrogel-forming salt selected from the group consisting of aluminum, tin and iron salts; silicic acid, a depressant for the insolubles selected from the group consisting of starch, glues, caramel, and caustic extracts of coal; a lime depressant selected from the group consisting of alkali pyrophosphates and sodium lignin sulfonate; and a collector reagent selected from the group consisting of oleic, palmitic, stearic, capric, lauric and naphthenic acids and their salts.

23. The process of treating magnesite ores by froth flotation, which comprises forming a magnesite ore pulp containing high grade magnesite, dolomite and low grade magnesite particles, introducing aluminum sulfate into the pulp to react with the dolomite particles and form calcium sulfate and a hydrogel, and selectively floating the high grade magnesite away from the dolomite reaction product in an alkaline medium having a pH of at least 8 by aerating the pulp in the presence of a collector reagent selected from the group consisting of oleic, palmitic, stearic, capric, lauric and naphthenic acids and their salts.

24. The process of treating magnesite ores by froth flotation, which comprises forming a magnesite ore pulp containing high grade magnesite and other particles containing calcareous constituents, introducing aluminum sulfate into the pulp to react with the calcareous particles and form calcium sulfate and a hydrogel, and selectively floating high grade magnesite away from the calcareous reaction product in an alkaline medium having a pH of at least 8 by aerating the pulp in the presence of a collector reagent selected from the group consisting of oleic, palmitic, stearic, capric, lauric and naphthenic acids and their salts.

25. The process of treating magnesite ores by froth flotation, which comprises forming a magnesite ore pulp containing high grade magnesite intermixed with a quantity of lime and insoluble constituent particles, and floating high grade magnesite selectively away from such lime and insoluble content of the pulp by aerating said pulp in the presence of: a hydrogel-forming salt selected from the group consisting of aluminum, tin and iron salts; polymerized silicic acid, a depressant for the insolubles selected from the group consisting of starch, glues, caramel, and caustic extracts of coal; a lime depressant selected from the group consisting of alkali pyrophosphates and sodium lignin sulfonate; and a collector reagent selected from the group consisting of oleic, palmitic, stearic, capric, lauric and naphthenic acids and their salts.